

Sept. 18, 1945.

W. E. SILLICK

2,384,853

PREPARATION OF WOOD PULP CELLULOSE FOR NITRATION

Filed Feb. 24, 1943



FIG.2



WILLIAM E. SILLICK

INVENTOR

*N. M. Perrins*  
BY *Daniel J. Mayne*  
ATTORNEYS

Patented Sept. 18, 1945

2,384,853

# UNITED STATES PATENT OFFICE

2,384,853

## PREPARATION OF WOOD PULP CELLULOSE FOR NITRATION

William E. Sillick, Rochester, N. Y., assignor to  
Eastman Kodak Company, Rochester, N. Y., a  
corporation of New Jersey

Application February 24, 1943, Serial No. 476,980

5 Claims. (Cl. 260—222)

This invention relates to a method of preparing wood pulp cellulose for nitration in which the wood pulp, in a disintegrated or loosely fibrous form, is subjected to a rolling action to form lightly compacted rods or "worms" of the cellulose.

The form which cellulose should take for nitration processes, particularly in processes of nitrating wood pulp, has been a subject for much investigation. Some investigators in this field have suggested a method of nitrating wood pulp by immersing wood pulp sheets directly in nitrating acid. Other have suggested formation of the wood pulp into chips and treating those chips with nitrating acid. Various other physical forms for wood pulp to be nitrated have been suggested, such as small bits, dust, or loosely separated fibers. Some of these physical forms of wood pulp are adapted only for the preparation of high viscosity cellulose nitrates. Other of the suggested forms of pulp have never been found to be suitable in nitrating processes because of the difficulty of penetration of the acid throughout the mass of cellulose. Still other of the suggested forms have been objectionable because of the bulkiness, dustiness, and absorbency resulting in diminished production with a given amount of equipment and, also, necessitating the use of a considerable excess of acid to promote the nitration processes.

The disintegration of wood pulp into a bulky mass of separated fibers, described in disclosures such as British Patent 336 of 1891, U. S. Patent 480,588, or German Patent 300,844, has resulted in material which has exhibited desirable properties in various nitrating processes. This disintegrated material, however, does have the disadvantages of dustiness and, because of bulkiness, necessitates large bins for a given weight. Also for certain nitrating processes in which the absorption of acid should be only moderate this material has not worked out so well. Although this disintegrated material is completely penetrated by a nitrating acid, because of the separation of the wood pulp into substantially individual fibers, nevertheless, bulkiness or dustiness results which apparently has ruled out this disintegrated pulp for nitrating purposes to any substantial extent. Few, if any, commercial processes at the present time use a bulky disintegrated wood pulp as the material to be nitrated.

An object of my invention is to provide a wood pulp cellulose having a physical form suitable for use in any of the ordinarily employed nitrat-

ing processes, whether to prepare high or low viscosity nitrate and whether to prepare a highly nitrated cellulose, such as of the gun cotton type, or a less highly nitrated cellulose, such as adapted for the preparation of sheeting or photographic film base. Another object of my invention is to prepare a wood pulp cellulose having advantages as to bin capacity, lack of dustiness, and ease of loading into the nitrating facilities. A still further object of my invention is to employ for a nitrating process a cellulose in a physical form in which the absorption of acid is such as to permit the use of relatively low ratios of acid to cellulose in the nitration tanks, such as less than ordinarily employed in the nitrating of cotton linters.

I have found that the various disadvantages residing in the use of a loosely fluffed wood pulp for nitrating purposes may be substantially eliminated by subjecting that fluffed material to a rolling action such as by subjecting it to the action of two surfaces either (1) moving in opposite direction, (2) one stationary and the other moving, or (3) both moving in the same direction but at different rates of speed. This action forms the cellulose into lightly compacted rods or "worms" having but a small diameter and a length several times the diameter, thus making for a large number of long rolled units. These units fit well together in a nitrating pot, exhibit little, if any, dustiness, and are uniformly penetrated by the nitrating acid without soaking up that acid to an undesirable degree. This formation of rolls or the so-called "worms" may, for example, be accomplished by spreading a fluffed wood pulp cellulose in a thin layer upon a surface and passing a cloth sheet, such as flannel, which cloth sheet presses down on the cellulose, thereover at a rate of speed different from that of the surface upon which the wood pulp is deposited.

In the accompanying drawing Fig. 1 illustrates an apparatus adapted for the preparing of the wood pulp rolls in accordance with my invention. 1 and 2 are each endless belts of the width desired, such as 18 inches or 2 feet up to 6 feet or more, moving in the same direction. The belt 1 is moved at a more rapid rate than endless belt 2, such as for instance, 20 to 40 feet per minute compared to a speed of 10 to 20 feet per minute for endless belt 2. Ducts 3 are for the purpose of admitting fluffed wood pulp cellulose to the endless belts as shown, while conveyor 4 receives the rods or "worms" after their formation and carries them through a drier or directly

to their storage bin. The supporting rollers shown are preferably adjustable so that the distance between the belts 1 and 2 may be adjusted, depending upon the density of the pulp which is fed in and the depth of the layer which is formed on belt 2 before being led through the rolling portion of the machine.

Fig. 2 is a plan view of a section of the conveyor 4 illustrating the carrying of the rods or "worms" thereby. In practice the units would preferably be more densely associated than shown. This combination of apparatus is given to illustrate a setup which has been found to be suitable for the purpose at hand. Obviously, other combinations involving the use of two surfaces moving at different rates may be employed to form the fluffed pulp into rods or rolls in accordance with my invention.

A fluffed cellulose which is quite suitable for use in the formation of rolls in accordance with my invention may be obtained, for instance, by passing pulp sheet (which is a usual form in which wood pulp is marketed) into a disintegrating apparatus such as a Sprout-Waldron attrition mill or an apparatus such as shown in British Patent 336 of 1891 or in U. S. Patent 480,588 of Kellner. Any apparatus which fluffs the cellulose into its individual fibers is suitable for preparing the fluffed wood pulp which may be employed. If desired, even cotton may be treated in accordance with my invention to impart the form of small rolls thereto. As the cellulose which is preferably employed in nitrating processes for making some types of nitro-cellulose has a high  $\alpha$ -cellulose content, in these cases it is desirable that the wood pulp which is employed as the starting material, in accordance with my invention, be a high  $\alpha$ -cellulose of good color with but a small proportion of impurities therein. In cases where color is not important, ordinary unbleached or partially bleached pulp may be employed. The pulp employed for nitrating is either sulfite or kraft pulp. Either of these may be used in the method of my invention.

One type of nitrating process to which my invention may be adapted is that described and claimed in U. S. Patent 2,118,275 for the making of cellulose nitrate which is nitrated to a nitrogen content of approximately 11.5 to 12.3%, particularly where a low viscosity cellulose nitrate is desired. After fluffing a high  $\alpha$ -cellulose wood pulp and forming it into rods or "worms" as described herein, these may be employed as the starting material for the nitration described in that patent. If a highly nitrated cellulose is desired the cellulose material prepared in accordance with my invention in the form of rods or rolls may be employed as the starting material in any of the processes ordinarily employed for that purpose; for instance, by utilizing a nitrating mixture comprising 28% nitric acid, 55% sulfuric acid, and 17% water the cellulose in the form imparted in accordance with my invention will not mat or form dense masses in the nitrating apparatus, nor will there be any dustiness or loss of cellulose resulting from handling. Also, the operations of stabilizing and dehydrating the nitrated wood pulp may be handled with facility, the product not being bulky or difficult to treat. Various forms of cellulose, as suggested in the prior art, are adapted to various types of nitration. For instance, some forms of cellulose suggested would only be suitable for the preparation of high viscosity cellulose nitrate. Other forms of cellulose would not be suitable for

processes in which a highly nitrated product is obtained. The rolls of cellulose or "worms," such as prepared in accordance with my invention, however, are adapted for various types of nitrating processes and will be found to be economical in that a relatively low ratio of acid to cellulose may be employed in the nitrating pot.

As an example of forming a cellulose nitrate in accordance with my invention, a sulfite pulp having a high  $\alpha$ -cellulose content and in sheet form, was passed through a disintegrating machine which fluffed the pulp, producing a material having a bulk value of 1200 units, nitration grade cotton linters being taken as 800 units, these units being based on volume per unit weight. This fluffed cellulose was then spread on a cloth-covered table in a layer about 1½ inches thick and the layer was rolled under a firm cloth-covered surface for a distance of about 9 feet with a pressure upon the pulp layer of about 10 pounds per square foot. The layer of cellulose formed a number of individual portions having a round, rodlike form and in this form were compacted and oriented into round, rodlike units about ¾ inches in diameter and 12-18 inches in length, and having definite properties of rigidity and tenacity so that they would withstand the normal rough handling of drying, conveying and weighing without appreciably losing their original compact form and without freeing an appreciable amount of dust. The bulk value of the cellulose was reduced from about 1200 units to about 700 units. This reduction in bulk was sufficient to yield a material which was easily handled in standard weighing containers and which could be charged into the nitrating vessels at normal rates of speed with no difficulty from floating or firing. The cellulose material was nitrated in accordance with the method described in U. S. Patent 2,118,275 of Talbot referred to above, and the final product, after washing, stabilizing, and dehydrating, was found to have characteristics satisfactory for a product of this kind.

It is desirable in passing the fluffed pulp in layer form between surfaces in accordance with my invention, that a moderate amount of pressure be exerted thereon. It is desirable that these surfaces be adjustable so as to control the spacing of these surfaces, depending on the thickness of the layer passed therethrough. Also by this means the degree of compactness of the rods or rolled units may be regulated. Ordinarily a pressure selected from the range 2-30 pounds per square foot will be most suitable as the density of the fluffed pulp is substantially decreased thereby without excessive compacting. If the pressure is too great the amount of compacting will be such that penetration of the rolled units by the nitrating acids will be difficult. If, on the other hand, too slight a pressure is employed very little compacting results and the valuable features of my invention will not be realized to the full extent.

Ordinarily cloth surfaces are quite suitable for preparing the rolled pulp in accordance with my invention. For instance, flannel, canvas, or some other cloth especially of good wearing qualities is suitable for use. The surfaces, however, may be of any material sufficiently rough that sliding does not occur, which would defeat the object of the invention.

Although the drawing shows rolls to impart rigidity to the cloth surfaces pictured there, other elements having this effect, such as plates or

boards presenting a smooth, rigid surface, may be employed instead. It is desirable that the pulp be dried after the passing between surfaces rather than before, as I have found the pulp behaves better in rolling into rodlike units when not completely bone-dry.

I claim:

1. The method which comprises passing a uniformly, loosely fluffed air-dry wood pulp having a bulk value of approximately 1200 units between surfaces having motion relative to each other, which lightly press upon the pulp so as to form the pulp into dry, loosely rolled units having a bulk value approximating 700 units.

2. A method of preparing cellulose nitrate from wood pulp, which comprises passing dry wood pulp sheet through a disintegrating mill to uniformly, loosely fluff pulp to a bulk value of approximately 1200 units, passing the uniformly, loosely fluffed air-dry pulp thus obtained between surfaces having motion relative to each other, which lightly press upon the pulp, to form the pulp into dry, loosely rolled units having a bulk value approximating 700 units and nitrating the dry, loosely rolled units thus obtained.

5 3. The method which comprises passing a uniformly, loosely fluffed air-dry wood pulp having a bulk value of approximately 1200 units between surfaces moving in opposite directions which lightly press upon the pulp so as to form the pulp into dry, loosely rolled units having a bulk value approximating 700 units.

10 4. The method which comprises passing a uniformly, loosely fluffed air-dry wood pulp having a bulk value of approximately 1200 units between surfaces one of which is stationary and the other moving, which surfaces lightly press upon the pulp so as to form it into dry, loosely rolled units having a bulk value approximating 700 units.

15 5. The method which comprises passing a uniformly, loosely fluffed air-dry wood pulp having a bulk value of approximately 1200 units between surfaces moving in the same direction but at different rates of speed, which surfaces lightly press upon the pulp so as to form it into dry, loosely rolled units having a bulk value approximating 700 units.

WILLIAM E. SILLICK.